

March 9, 1937.

W. P. COHOE

2,072,943

TRANSFER MEDIUM AND METHOD OF MAKING SAME

Filed Nov. 30, 1935



*Fig. 1.*



*Fig. 2.*

INVENTOR  
*Wallace Patten Cohoe.*  
BY  
*L. S. Julian*  
ATTORNEY

## UNITED STATES PATENT OFFICE

2,072,943

TRANSFER MEDIUM AND METHOD OF  
MAKING SAME

Wallace Patten Cohoe, New York, N. Y., assignor,  
by mesne assignments, to Underwood Elliott  
Fisher Company, New York, N. Y., a corpora-  
tion of Delaware

Application November 30, 1935, Serial No. 52,282

5 Claims. (Cl. 91—68)

This invention relates to a transfer medium and to a method of manufacturing the same. More particularly it relates to carbon webs or sheets, such as are extensively used for manifolding in typewriters and various other business machines, and to an improved method of manufacturing such webs or sheets to provide the advantages hereinafter set forth.

Such webs and sheets are commonly made of a paper base faced with a transfer coating composition of comminuted carbon, coloring ingredient, carnauba wax and petroleum jelly. According to the particular use in view they are made of varying weights of paper stock and varying 15 degrees of hardness of the transfer material used as a coating and each variation may have special applicability to some particular field of use and be in a measure unsuited to other uses. Each variation presents its own particular problems of 20 manufacture but substantially all of them are subject to the common objection that under certain atmospheric conditions they tend to curl from the edges in the direction of the transfer facing and under some conditions curl into a roll 25 making the use of the same difficult or in some instances impossible.

Another objection to transfer sheets now largely in commercial use is that owing to the smooth surface of the uncoated back of the paper, there is difficulty in obtaining and maintaining good alignment and registration of the components of the manifolding set because of the tendency of the interleaved transfer sheets to slip 30 from position.

It is an object of the present invention to remove these objections and provide a transfer sheet that will be substantially non-curling in character and both front and back surfaces of which are treated to prevent the tendency to slip 35 from registered position. Other objects will appear as the description of this invention proceeds.

The reason for the curling tendency of transfer sheets is defined as due to unequal expansions 40 between the paper base or body of the sheet and its wax and carbon facing. The paper which is a felted mass of hydrated cellulose fibres has a hydroscopic characteristic whereas the wax and carbon coating at the face of the paper is com- 45 paratively impervious to atmospheric moisture changes. At times of high humidity the paper base will take up moisture from the atmosphere and expand and the relative difference in expansion between the base and the coating brings 50 about the well-known result of curling in analogy

to that so clearly apparent in bimetal thermo-  
static devices.

Curling of transfer sheets appears to be caused, also, to some extent, from the uneven stresses set up in the facing of the paper when the transfer coating is applied in molten form and solidified. There is some impregnation by the molten wax composition of a substratum of the paper and the contraction of the facing of the paper attendant upon the solidification of the coating sets up stresses which are retained for some period of time until a natural rearrangement takes place which in a measure relieves the initial stresses. It is believed, however, that whatever amount of seasoning time is given to the coating paper there 10 always remains some stresses in the coating which have a tendency to distort to some extent the edges of the paper. Apparently there is always a tendency of the coating to remain stationary or to contract unless, of course, the paper is subjected to considerable heat. Obviously, 15 with these tendencies present in the transfer coating, whatever moisture is taken up by the paper base tends to cause curling of the sheet.

Sheets or webs treated with a facing of coating 20 material, have heretofore been coated on their reverse or rear surfaces with compositions or solutions of various kinds. Such reverse coatings have been applied with the end in view of increasing the resistance of the paper to the blows of the type, that is, to toughen it or give it mechanical reenforcement purely. Papers having wax 25 coated back surfaces have found some small sale commercially but have not attained any large measure of popularity because of their failure to satisfactorily meet the range of manifolding requirements. So far as is known, no such reverse-coated paper has been made by which as good 30 manifolding can be obtained under all conditions as with an ordinary carbon sheet untreated at the back surface. In the use of such sheets, the writes of the first copies will lack the desirable sharpness and if a large number of copies are 35 to be produced simultaneously, those following the first two or three are illegible.

By the present invention a transfer sheet is 40 produced which is substantially non-curling at all room temperatures, which has characteristics of durability and longevity and in which there is no sacrifice in sharpness of write or legibility of all 45 copies of the manifolding set and in which, as a matter of fact, it has been observed by comparison that the first writes in the manifolding set have 50 sharpness superior to the first writes of a set employing unbacked sheets.

In the accompanying drawing:—

Figure 1 is a view in cross-section, greatly enlarged, of a fragment of a face-coated transfer sheet and illustrates a primary step in the method 5 of making a transfer sheet according to this invention.

Figure 2 is a similar view illustrating a subsequent step in the method and illustrative of the completed product.

10 The first part of the method which is employed in carrying out the present invention differs in no material respect from the conventional manner of making a carbon-faced web according to known practice. A paper web is run from a roll 15 through the feed rollers of a conventional coating machine and a transfer coating of a composition of comminuted carbon or other pigment or dye with wax and a fatty material such as petroleum jelly, is applied in a molten condition to one 20 side of the paper. The coating is solidified, and appears substantially as indicated at 10 in the drawing, upon and to some extent impregnating the paper stock 11. The paper web is then run again through the same or a similar machine 25 and a reverse or back coating 12 is applied.

The coating 12 is of chlorinated rubber or some 30 material having substantially like properties. Preferably it is applied as a solution of chlorinated rubber of the range 5 to 20% in toluol, the percentage varying within approximately this 35 range according to the degree of hardness of the transfer coating on the particular web and the purposes intended to be served by the sheets cut therefrom. Any suitable plasticizer may be included in the solution such as a vegetable oil or resin, approximately 5%, and fillers and pigments or dyes may be included if desired.

For the purpose of preventing curl and minimizing the objectionable slipping characteristic 40 of the paper, it has been found that a solution of 5% chlorinated rubber in toluol is suitable. In cases where durability and sharpness of first writes are more important than manifolding properties it is preferred to use higher percent- 45 ages of chlorinated rubber.

The solution may be applied according to any 50 of the usual methods as, for example, by spraying, brushing or flowing, and the excess over desired amount is removed by a knife or other conventional gaging or levelling means. The solvent is then evaporated and the paper is subsequently rolled.

Chlorinated rubber as commercially produced in high chlorine content is of such specific gravity and density that its application to a thin web 55 of carbon-faced paper adds materially to the weight, resistance and sensitiveness of the paper without unduly increasing its bulk. Furthermore the chlorination of the rubber so lowers 60 its viscosity that it can be made to run in almost water-thin solution to spread easily and evenly and impregnate the paper to some extent, yet it is highly cementitious and effective for the desired purposes. The high mobility of the chlorinated rubber in solution has a distinct importance to this invention. The specific gravity of chlorinated rubber according to present proc-

esses may be 1.5 and the chlorine content may run as high as 60 to 70%. Solutions of few percent of caoutchouc are difficult to flow whereas the higher percentages of chlorinated rubber with high solids content may be readily flowed and spread in an extremely thin yet relatively dense moisture-resistant film on the back of the thin paper web previously coated on its face with a moisture-resistant transfer coating.

Furthermore, the chlorinated rubber backing 10 is corrective of curl produced in previously known carbon papers by cool atmospheric temperature which contracts the carbon coating more than its paper base, causing a carbon concave curl. This type of curl has not been corrected by coatings of gutta-percha which have been attempted. The use of gutta-percha was intended for toughening the sheet.

According to a preferred method employed, the 20 solution of chlorinated rubber in toluol is applied after the wax and carbon transfer-coating has been applied and solidified, for the reason that by first applying and solidifying the wax coating the paper web is reenforced and held to a large extent against longitudinal stretching in the 25 coating machine.

The final product derived from this invention is a thin flexible sheet, soft but resilient and sensitive, stable under all room temperature conditions and provided with a backing which is a 30 moisture-resistant deposit of chlorinated rubber from an evaporation of the solvent in a solution of the same and which consequently has substantial weight and density to prevent curling of the paper and add to its mechanical strength, 35 durability and manifolding properties. The backing of the sheet is unaffected by atmospheric changes. It is of excellent appearance with a slight lustre and it is just sufficiently tacky to assist in maintaining the sheet in position in 40 the manifolding set.

What I claim as new, is:—

1. A transfer web having on its face a transfer material and on its back a thin dense film of chlorinated rubber.

2. A paper sheet having on its face a transfer material and on its back a thin dense coating of chlorinated rubber.

3. The method of making a transfer sheet which comprises applying to one side of a paper web a transfer coating of carbon carried in a waxy substance thus reenforcing the paper against stretch when wet, and applying chlorinated rubber in solution to the other side of the web and evaporating the solvent.

4. The method of making a transfer sheet which comprises applying a transfer coating to one side of a roll-fed paper web, applying chlorinated rubber in solution to the other face of the web, removing excess of the solution, and evaporating the solvent.

5. A non-curling carbon-paper sheet having on its face a transfer material comprising comminuted carbon in wax and a fatty substance, and having chlorinated rubber on its back.

WALLACE PATTEN COHOE.